# EUROPEAN PATENT SPECIFICATION

(11) **EP 2 923 856 B1**
(45) Date of publication and mention of the grant of the patent: **18.10.2017**
(21) Application number: 13856068.5
(22) Date of filing: 28.06.2013
(51) Int. Cl.: B44C 1/175, B05D 5/06, B05C 1/02, B05C 1/08, B05D 7/14, B05D 7/00, B05D 1/28, B05D 1/36, B41F 33/00, B41F 17/00

(54) **METHOD OF PRODUCING VARIEGATED STEEL PLATE WITH MULTICOLOURED PATTERN**
VERFAHREN ZUR HERSTELLUNG EINER VARIEGIERTEN STAHLPLATTE MIT VIELFARBIGEM MUSTER
PROCÉDÉ DE PRODUCTION D'UNE PLAQUE EN ACIER MARBRÉE AVEC UN MOTIF MULTICOLORE

(30) Priority: 23.11.2012 CN 201210481610
(43) Date of publication of application: 30.09.2015
(73) Proprietor: Liaoning Chaoshuo Toma Technology Steel Plate Printing Co. Ltd., Liaoning 115000 (CN)
(72) Inventor: TANG, Yueping, Yingkou Liaoning 115000 (CN); ZHOU, Jianping, Yingkou Liaoning 115000 (CN); WU, Liang, Yingkou Liaoning 115000 (CN)
(74) Representative: Groth & Co. KB
(86) International application number: PCT/CN2013/078368
(87) International publication number: WO 2014/079214

(56) References cited:
- CN-A- 101 912 839
- CN-A- 102 991 113
- CN-A- 102 991 123
- CN-A- 103 147 670
- CN-A- 103 158 339
- CN-A- 103 158 380
- CN-A- 103 158 381
- CN-A- 103 158 415
- CN-U- 202 965 490
- CN-Y- 201 283 692
- JP-A- 2005 288 936

## Description

### FIELD OF INVENTION

The present invention relates to a method for producing variegated steel plate with multicoloured patterns, in particular, a method of producing variegated steel plate with multicoloured patterns, belonging to the field of variegated steel plate manufacturing.

### BACKGROUND OF THE INVENTION

Coloured coating steel plate (commonly known as variegated steel plate) refers to that a metal substrate is treated by surface pretreatment prior to painting such as surface degreasing treatment and surface passivating treatment through a continuous unit, and then is coated with one-layer or multilayer of organic coatings on the surface, thus forming a composite material.

In order to coat multicoloured patterns, the colour of coating is required to be changed for several times a day for a majority of coating production line, and in order to realize the purpose of non-stop production, non-decrease yield and quick colour change, generally two devices for fine coating are arranged at the front position of coating layer of the machine for fine coating of the processing line, characterized in that, device 1 is a single-head device for fine coating, and device 2 is a dual-head device for fine coating, which is arranged under machine 1, and when one device for fine coating coats a strip steel, the other one prepares for printing the next colour, however, the above processing line is lack of a positioning system used for determining a relative position of various colour, which is just used for coating a regular pattern, but cannot produce an irregular one.

The intaglio printing machine used in the prior art of roller coating type for producing variegated steel plate with multicoloured patterns comprises a feeding equipment, used for providing paints; a suction roller, whose circumferential surface is in connection with the feeding equipment, and has a plurality of recesses adapted for being filled with paints for forming an image area; and a coating roller, with its circumferential surface in connection with the suction roller, and used for receiving and transferring the image area formed by the paints on the coating roller onto a steel plate to form desired multicoloured patterns. CN 101 912 839 A discloses a continuous processing method of printed color coated steel plates at normal temperature, which comprises the following steps : A) uncoiling and butting; B) degreasing and cleaning; C) carrying out passivation treatment; D) coating a primer layer; E) printing at the normal temperature; and F) coating a finish coat layer. However, during the process of using the intaglio printing machine, the applicant found out that the roller surface linear velocity of the suction roller and the rubber coating roller are frequently inconsistent with the process speed of the whole production line, and the whole production line is lack of a control system for on-line adjusting the rotation speed of the suction roller and the rubber coating roller, so the whole production line has to be stopped for adjustment after operation for a period of time, thus affecting the efficiency of the whole production line. If the production line is not stopped for adjustment, the steel strip transporting speed would be inconsistent with the roller surface linear velocity of each roller, thus frequently causing the steel strip unable to be coated at a designated position thereof. Besides, in order to print multicolour patterns, a plurality of roller coating units are required for coordinated operation. However, the above mentioned intaglio printing machine in the prior art is lack of a control system for allowing a continuous production between adjacent roller coating units, so workers need observe by human eyes if a first roller coating unit has completed coating of one colour, and if yes, an adjacent roller coating unit will be started by manual work, thus it is unable to realize a continuous production between the adjacent roller coating units. At the same time, due to lack of the control system for adjusting the speed, it is unable to realize error revision when misplacement occurs between the patterns printed by the adjacent roller coating units.

### SUMMARY OF THE INVENTION

Therefore, a first technical problem to be solved by the present invention is to provide a method of producing variegated steel plate with multicoloured patterns, by which the rotation speed of each roller of a roller coating unit is able to be adjusted to be consistent with the rotation speed of the process, thus improving the production efficiency.

A second technical problem to be solved by the present invention is to provide a method of continuously producing variegated steel plate with multicoloured patterns on the processing line of adjacent roller coating units.

A third technical problem to be solved by the present invention is to provide a method of producing variegated steel plate with multicoloured patterns which are lifelike and complete, because it is able to conduct error revision when misplacement occurs between the patterns.

In order to solve at least one of the above mentioned technical problems, in a class of embodiments, the present invention provides a method of producing variegated steel plate with multicoloured patterns, comprises the following process steps in sequence: A. preparing a steel strip to be printed; B. using a first roller coating unit to perform a first roller coating transfer on the steel strip to be printed; C. using a second roller coating unit to perform a second roller coating transfer on the steel strip to be printed after a specific time; in the step B, a servo control system is used to control the first roller coating unit, and the servo control system has a following control process: S1. data of diameter of each roller and a process speed of the first roller coating unit are input into a PLC control module, then the PLC control module calculates out theoretical roller surface linear velocity of each roller according to the process speed and the diameter of each roller, allows the theoretical roller surface linear velocity of each roller to be consistent with the process speed, and outputs the calculated theoretical roll surface linear velocity signal of each roller into a servo control module having an encoder; S2. the servo control module receives the theoretical roll surface linear velocity signal of each roller from the PLC control module and drives each roller according to the signal; S3. the encoder collects actual roller surface linear velocity of each roller and outputs the actual roller surface linear velocity signal of each roller into the PLC control module; S4. according to the received actual roller surface linear velocity signal and theoretical roller surface linear velocity signal of each roller, the PLC control module adjusts current frequency of electrical machine driving each roller, and adjusts the actual roller surface linear velocity of each roller to be consistent with the theoretical roller surface linear velocity of each roller, and then the roller coating transfer of the first roller coating unit is completed; in the sub-step S1 of step B, distance data between the first roller coating unit and the second roller coating unit is input into the PLC control module, and on the basis of the process speed and the distance data, the PLC control module calculates out a specific time to start the second roller coating unit, and starts the second roller coating unit according to the specific time, and then the second roller coating transfer of the second roller coating unit is completed.

In a class of this embodiment, after the sub-step S4 of step B, the printed pattern is collected by a code recognition module, and the pattern misplacement distance is determined by computer recognition, and then the process speed of the corresponding roller coating unit is revised.

In a class of this embodiment, in the step A, using an decoiler to decoil and trim the steel strip and using a seamer to seam the decoiled steel strip.

In a class of this embodiment, the method further comprises a step of pre-processing the steel strip to be printed before transferring between the step A and the step B.

In a class of this embodiment, the pre-processing before transferring comprises the following steps in sequence: degreasing treatment, cleaning treatment, first drying treatment, passivating treatment and second drying treatment.

In a class of this embodiment, after the second drying treatment, the steel strip is treated in sequence by coating primer paint treatment, baking for curing treatment, and first cooling treatment.

In a class of this embodiment, after step C, spraying the steel strip with gloss paint, followed by a third drying treatment, followed by a second cooling treatment.

In a class of this embodiment, a recoiler is used to coil the steel strip after completing all the roller coating transfer.

In a class of this embodiment, the roller coating unit used in the step B and step C comprises a feeding equipment used for providing paints; a suction roller, whose circumferential surface is in connection with the feeding equipment and has a plurality of recesses adapted for being filled with paints for forming an image area; a rubber-coating roller, with its circumferential surface in connection with the suction roller, used for receiving and transferring the image area formed by the paints on the coating roller onto a steel plate; a first scraper, arranged on a first scraper support and contacting with the suction roller at a specific angle, used for scraping off paints outside the image area on the suction roller; and a second scraper, arranged on the second scraper support and contacting with the coating roller at a specific angle, used for scraping off paints outside the image area on the rubber coating roller.

The method of producing variegated steel plate with multicoloured patterns of present invention providing has advantages as bellow:
1. in the method of producing variegated steel plate with multicoloured patterns of the present invention, for the first transfer, on one hand, the PLC control module of the servo control system collects the process speed and the rotation speed of each roller of the roller coating unit, calculates out the theoretical roller surface linear velocity and makes the theoretical roller surface linear velocity be consistent with the process rotation speed; on the other hand, the actual roller surface linear velocity of each roller of the roller coating unit is collected by a servo control module having an encoder, and the signal of the actual roller surface linear velocity is input into the PLC control system, so that the PLC control system can compare the actual roller surface linear velocity with the theoretical roller surface linear velocity, and adjust current frequency until the actual roller surface linear velocity is consistent with the theoretical roller surface linear velocity. In the above mentioned control method, the actual roller surface linear velocity is adjusted to be consistent with the theoretical roller surface linear velocity which is consistent with the process speed, thus ensuring that the actual roller surface linear velocity is consistent with the process rotation speed, so there is no need to stop the line for adjusting in the production process, thus increasing the production efficiency.
2. In the method of producing variegated steel plate with multicoloured patterns of the present invention, the distance data between the first roller coating unit and the second roller coating transfer unit is also input into the PLC control module, and on the basis of the process speed and the distance data, the PLC control module is able to calculate out a specific time to start the second roller coating unit. Once the production line is determined, the distance between adjacent units can be determined. The distance data is input into the PLC control module in advance, and then according to the process speed and distance data, the PLC control module calculates out the specific time to start next roller coating unit. Then the specific time to start next roller coating unit is able to be preset, and the next roller coating production line is allowed to be started within the specific time, so a continuous production between the adjacent roller coating units is realized, and the production efficiency is further improved.
3. The method of producing variegated steel plate with multicoloured patterns further comprises a code recognition module. The printed pattern is collected by the code recognition module, and the pattern misplacement distance is determined by computer recognition, and then the process speed of the corresponding roller coating unit is revised. After next roller coating production line is started and the second transfer is completed, the printed pattern is collected by the code recognition module and the pattern misplacement distance is determined by the computer recognition, and then the rotation speed of each roller is revised in accordance with the pattern misplacement distance, so that the pattern misplacement can be revised. The above process can be circularly performed, hence ensuring lifelike and complete printed patterns. In addition, the length of the printed patterns is extended greatly by using the code recognition module.

### BRIEF DESCRIPTION OF THE DRAWINGS

In order to make the present invention more easily and clearly understood, the invention is further described below in conjunction with the detailed embodiments and the drawings, characterized in that,
Figure 1 is a flow chart of a method of producing variegated steel plate with multicoloured patterns of the present invention;
Figure 2 is a schematic view of a roller coating unit of the present invention;
Figure 3 is a workflow chart of a servo control system provided by the present invention;

The reference numbers in the drawings represent:
1-feeding equipment; 2-suction roller; 3-rubber coating roller; 4-first scraper; 5-second scraper; 6-cleaning device; 61- liquid feed tank; 62- transfer pump; 63-transfer pipe; 64-spay pipe; 65-spay hole; 67- recovery tank; 68- filter; 7-support roller

### DETAILED DESCRIPTION OF THE EMBODIMENTS

### Embodiment 1

As shown in Figure 1, this embodiment provides a method of producing variegated steel plate with multicoloured patterns, comprising the following process steps in sequence:
A. preparing a steel strip to be printed;
B. using a first roller coating unit to perform a first roller coating transfer on the steel strip to be printed;
C. using a second roller coating unit to perform a second roller coating transfer on the steel strip to be printed after a specific time.

In the step B, a servo control system is used to control the first roller coating unit, and the servo control system has a following control process as shown in Figure 3:
S1. data of diameter of each roller and a process speed of the first roller coating unit are input into a PLC control module, whereby the PLC control module calculates out theoretical roller surface linear velocity of each roller (Computational formula of theoretical rotation speed: theoretical rotation speed = process speed /π* diameter of each roller, and PLC control module calculates out the theoretical rotation speed firstly and then determines the theoretical roller surface linear velocity according to the theoretical rotation speed: theoretical roller surface linear velocity = theoretical rotation speed* roller diameter *π), allows the theoretical roller surface linear velocity of each roller to be consistent with the process speed, and outputs the calculated theoretical roll surface linear velocity signal of each roller into a servo control module having an encoder;
S2. the servo control module receives the theoretical roll surface linear velocity signal of each roller from the PLC control module and drives each roller according to the signal;
S3. the encoder collects actual roller surface linear velocity of each roller and output the actual roller surface linear velocity signal of each roller into the PLC control module;
S4. according to the received actual roller surface linear velocity signal and theoretical roller surface linear velocity signal of each roller, the PLC control module adjusts current frequency of electrical machine driving each roller, and adjusts the actual roller surface linear velocity of each roller to be consistent with the theoretical roller surface linear velocity of each roller, and then the roller coating transfer of the first roller coating unit is completed.

In the present embodiment, in order to realize continuous operation of adjacent roller coating units on line, in the sub-step S1, distance data between the first roller coating unit and the second roller coating unit is input into the PLC control module, and on the basis of the process speed and the distance data, the PLC control module calculates out a specific time to start the second roller coating unit, and starts the second roller coating unit according to the specific time, and then the second roller coating transfer of the second roller coating unit is completed.

In the present embodiment, in order to print irregular long patterns, after completing the printing of the second roller coating unit, that is, after the step S4, the printed patterns are collected by a code recognition module, and the pattern misplacement distance is determined by a computer recognition system, and then the process speed of the corresponding roller coating unit is revised. The revision process is described in detail as below. If the actual position of a latter printed colour in the patterns collected by the code recognition module misplaces a distance from the predetermined position of the latter printed colour relative to the former printed colour , for example, the actual position locates at 10mm ahead of the predetermined position, which indicates that the actual process speed (denoted by V1) of the roller delivering the steel strip speeds up 10mm per unit time relative to the theoretical process speed (denoted by V2), that is at this time, V2=V1-10, thus calculating out V2. Then the calculated V2 is converted into the theoretical rotation speed of the roller (denoted by N) via the formula N=V2/π*roller diameter, thereby adjusting the current frequency of the corresponding electric machine in accordance with rotation speed N, thus the rotation speed of the corresponding roller will be adjusted, and the process speed will be further adjusted, and finally the pattern misplacement accuracy is controlled within ±0.6 millimeter. This adjusting process is a dynamic and repeated process. Herein, the printed patterns are collected by a digital video comprised in the code recognition module.

In order to improve the formability of the printed steel strip, the present embodiment preferably comprises a step of pre-processing the steel strip to be printed before transferring between the step A and step B, and the pre-processing before transferring comprises the following steps in sequence: in the degreasing treatment, an alkali liquor with an concentration of 1% and an temperature of 50-65 degrees is used to perform degreasing so as to remove oil and dust from the surface of the strip steel, and in the alkali liquor, the ratio of total alkali to free alkali is less than 2.5; in the cleaning treatment, desalted water having a temperature of 50-65 degrees and a PH value less than 7.8 is used to wash the surface of the strip steel after degreasing treatment, so as to remove residual alkali liquor on surface of the strip steel; in a first drying treatment, hot air having a temperature of 75-85 degrees heated by a vapor heat exchanger is used to dry the surface of the strip steel after cleaning so as to remove residual water thereon; in the passivating treatment, the surface of the strip steel after cleaning is passivated with a treating solution having Chromium weight of 22-32, so as to increase the adhesion force between the strip steel and the primer paint and also increase the antiseptic property; in a second drying treatment, the passivated surface is dried by an electrical heating oven at a baking temperature of 75-85 degrees, in order to enhance passivation effect. In the coating primer paint treatment, the first roller coating unit is used to coat primer paint and back paint on the surface of the strip steel, and the colour and the property of the primer paint depend on the patterns to be printed; in the baking for curing treatment and first cooling treatment, the strip steel coated with the primer paint and the back paint is baked to allow the primer paint and the back paint to be fully dried at temperature of 214-232 degrees, then the strip steel is cooled by water spay and flow to further stabilize the property of the primer paint and the back paint.

In the present embodiment, in order to improve brightness of the patterns and protection for the pattern, a post processing treatment is performed to the steel strip in the step C, and the post processing treatment comprises steps of spraying gloss paint on the surface of the steel strip, and then performing a third drying treatment, followed by a second cooling treatment.

In the present embodiment, in order to let the produced steel strip be convenient for storage and transport, a recoiler is used to coil the steel strip after completing all the roller coating transfer.

In the present embodiment, after the first roller coating transfer and after the first roller coating transfer, it further comprises a step of intermediate treatment which is drying and cooling treatment, and it should be noted that, the intermediate treatment should be ensured to complete before starting the second roller coating unit, alternatively, the time of performing the intermediate treatment is taken into consideration when calculating out the specific time to start the second roller coating unit, thereby revising the starting time of the second roller coating unit.

It should be noted that, for the production method of the above variegated steel plate with multicoloured patterns of the present invention, roller coating units are required for carrying out the step B and the step C, but there is no limitation to the specific structure of the roller coating units.

It should be noted that, the present embodiment provides a method for producing a variegated steel plate with two coloured patterns, which requires two roller coating units. While on the basis of the production method of the present embodiment, in particular of the techniques for adjusting rotation speed, time for starting the second roller coating unit, and the code recognition in the servo control system, modifications can be made by those skilled in the art so as to produce variegated steel plate with patterns in three-, four-, five- or more colours.

### Embodiment 2

The present embodiment provides a structure of the roller coating unit used in the steps B and C in the embodiment 1. As shown in Figure 2, the roller coating unit comprises a feeding equipment 1 used for providing paints; a suction roller 2, whose circumferential surface is in connection with the feeding equipment 1, and has a plurality of recesses adapted for being filled with paints for forming an image area; a rubber-coating roller 3, with its circumferential surface in connection with the suction roller 2, used for receiving and transferring the image area formed by the paints on the coating roller 3 onto a steel plate; a first scraper 4, arranged on a first scraper support and contacting with the suction roller 2 at a specific angle, used for scraping off paints outside the image area on the suction roller 2; and a second scraper 5, arranged on the second scraper support and contacting with the coating roller 3 at a specific angle, used for scraping off paints outside the image area on the rubber coating roller 3.

The working process of the roller coating unit in the present embodiment is described as below. The suction roller 2 runs, and the feeding equipment 1 supplies the suction roller 2 with paints. Apart of the paints gets into the recesses used for forming an image area on the suction roller 2, and another part of the paints locates outside the recesses on the suction roller 2. The paints outside the recesses on the suction roller 2 is scraped off by the first scraper 4, then the suction roller 2 rotates to transfer the paints in the recesses onto the rubber-coating roller 3 to form an image area. Then the paints outside the image area on the rubber coating roller 3 is scraped off by the second scraper, then the rubber coating roller 3 rotates to transfer the image area onto the metal plate to be printed to form a pattern. The metal plate to be printed is supported by a support roller 7 which also provides a supporting force for the coating operation of the rubber coating roller.

The present embodiment provides a method of producing variegated steel plate with multicoloured patterns as follows:
A. preparing a steel strip to be printed, characterized in that, using an decoiler to decoil and trim the steel strip and using a seamer to seam the decoiled steel strip;
B. using a first roller coating unit to perform a first roller coating transfer on the steel strip to be printed;
C. using a second roller coating unit to perform a second roller coating transfer on the steel strip to be printed after a specific time;

In the step B, a servo control system is used to control the first roller coating unit, and the servo control system has a following control process:
S1, the diameters of the suction roller 2 and the coating roller 3 and the process speed of the first roller coating unit are input into the PLC control module, then the PLC control module calculates out the theoretical roller surface linear velocity of the suction roller 2 and the coating roller 3 according to the process speed and the diameter of the suction roller 2 and the coating roller 3, allows the theoretical roller surface linear velocity of the suction roller 2 and the coating roller 3 to be consistent with the process speed, and outputs the calculated theoretical roller surface linear velocity signal of the suction roller 2 into a first servo control module having a first encoder, and outputs the theoretical roller surface linear velocity signal of the coating roller 3 into a second servo control module having a second encoder;
S2, the first servo control module receives the theoretical roller surface linear velocity signal of the suction roller 2 from the PLC control module and drives the suction roller 2 according to the signal; and the second servo control module receives the theoretical roller surface linear velocity signal of the coating roller 3 from the PLC control module and drives the coating roller 3 according to the signal;
S3, the first encoder collects the actual roller surface linear velocity of the suction roller 2 and outputs the actual roller surface linear velocity signal of the suction roller 2 into the PLC control module, and the second encoder collects the actual roller surface linear velocity of the coating roller 3 and outputs the actual roller surface linear velocity signal of the coating roller 3 into the PLC control module;
S4. according to the received actual roller surface linear velocity signal and the theoretical roller surface linear velocity signal of the suction roller 2 and the coating roller 3, the PLC control module adjusts current frequency of electrical machine driving each roller, and adjusts the actual roller surface linear velocity of the suction roller 2 and the coating roller 3 to be consistent with the theoretical roller surface linear velocity of the suction roller 2 and the coating roller 3, and then the roller coating transfer of the first roller coating unit is carried out and completed.

The rubber coating roller 3 of the roller coating unit of the present embodiment is made from rubber, and such a design of structure allows the rubber coating roller to flexibly contact with the suction roller 2 and the steel plate to be printed respectively, thus ensuring an exactly matching contact. In this way, the image area on the suction roller 2 can be completely transferred onto the rubber coating roller 3, and the image area on the rubber coating roller 3 can be completely transferred onto the steel plate to be printed, thus forming a complete image area. Moreover, the intaglio printing machine provided in the present embodiment comprises a first scraper 4 and a second scraper 5 (Figure 1 is a schematic diagram showing the first scraper 4 in contact with the suction roller 2 and the second scraper 5 in contact with the rubber coating roller 3). The first scraper 4 is used to scrape off the paints outside the recesses on the suction roller 2, and the second scraper 5 is used to scrape off the paints outside the image area on the rubber coating roller 3, thus avoiding the defect of lower labor efficiency caused by manual scrape, thereby improving labor efficiency. In addition, the first scraper 4 and the second scraper 5 are contacting with the suction roller 2 and the rubber coating roller 3 at a specific angle respectively, which can ensure better effect of scraping and prolonging the service life of the scraper.

It should be noted that, the coating roller may also be made from other materials as well as rubber, as long as the materials can ensure normal coating and flexible contact with the suction roller and the steel plate to be printed, such as silicone products which can meet requirements for elasticity, hardness and transfer property during coating.

In the present embodiment, the first scraper 4 contacts with the suction roller 2 at an angle less than 30 degrees, and the second scraper 5 contacts with the coating roller 3 at an angle more than 30 degrees. During intaglio printing process, paints that need to be scraped off are located on different positions at a same moment, so the first scraper 4 and the second scraper 5 are set at different angles, thus ensuring paints on the suction roller 2 and the coating roller 3 can be scraped off at the same time.

In the present embodiment, the first scraper 4 is made from titanium steel plate and has a blade thickness of 0.3mm, and the second scraper 5 is made from titanium steel plate and has a blade thickness of 0.3mm.

In the present embodiment, in order to improve the properties of the roller coating unit, a cleaning device 6 is provided for cleaning the paints on second scraper 5 and the rubber coating roller 3. The cleaning device 6 comprises a liquid feed tank 61, a transfer pump 62 used for pumping the cleaning liquid in the liquid feed tank 61, a cleaning liquid transfer pipe 63 communicated with the cleaning liquid transfer pump 62, and a spay pipe 64 communicated with the cleaning liquid transfer pipe. The spay pipe 64 is arranged above the rubber coating roller 3 in the axial direction and has a plurality of spay holes 65 thereon. The cleaning device 6 further comprises a cleaning liquid recovery tank 66, arranged below the coating roller 3 and connected with a recovery pipe 67 leading to the liquid feed tank 61. A filter 68 is arranged between the recovery pipe 67 and the liquid feed tank 61.

The working process of the cleaning device 6 provided in the present embodiment is described as below.

When at work, the cleaning liquid in the liquid feed tank 61 is pumped to the spay pipe 64 by the transfer pump 62, and is sprayed through the spray holes 65, subsequently the cleaning liquid flows over the rubber coating roller 3 and flows into the recovery tank 66, then passes through the recovery pipe 67 and is filtered by the filter 68, and finally gets back to the liquid feed tank 61 for recycling.

In the present embodiment, the feeding equipment 1 is a tray with a groove.

While particular embodiments of the invention have been shown and described, it will be obvious to those skilled in the art that changes and modifications may be made without departing from the invention in its broader aspects, and, therefore, the aim of the appended claims is to cover all such changes and modifications as fall within the scope of the invention.

## Claims

1. A method of producing variegated steel plate with multicoloured patterns, comprising the following process steps in sequence:
A. preparing a steel strip to be printed;
B. using a first roller coating unit to perform a first roller coating transfer on the steel strip to be printed;
C. using a second roller coating unit to perform a second roller coating transfer on the steel strip to be printed after a specific time;
in the step B, a servo control system is used to control said first roller coating unit, and the servo control system has a following control process:
S1. data of diameter of each roller and a process speed of said first roller coating unit are input into a PLC control module, then the PLC control module calculates out theoretical roller surface linear velocity of each roller according to the process speed and the diameter of each roller, allows the theoretical roller surface linear velocity of each roller to be consistent with the process speed, and outputs the calculated theoretical roll surface linear velocity signal of each roller into a servo control module having an encoder;
S2. the servo control module receives said theoretical roll surface linear velocity signal of each roller from the PLC control module and drives each roller according to the signal;
S3. the encoder collects actual roller surface linear velocity of each roller and outputs the actual roller surface linear velocity signal of each roller into the PLC control module;
S4. according to the received actual roller surface linear velocity signal and theoretical roller surface linear velocity signal of each roller, the PLC control module adjusts current frequency of electrical machine driving each roller, and adjusts the actual roller surface linear velocity of each roller to be consistent with the theoretical roller surface linear velocity of each roller, and then the roller coating transfer of the first roller coating unit is completed;
**characterized in that**, in the sub-step S1 of step B, distance data between the first roller coating unit and the second roller coating unit is input into the PLC control module, and on the basis of the process speed and the distance data, the PLC control module calculates out a specific time to start the second roller coating unit, and starts the second roller coating unit according to the specific time, and then the second roller coating transfer of the second roller coating unit is completed;
the roller coating transfer of the first roller coating unit and the second roller coating transfer of the second roller coating unit are used for printing multicoloured patterns on the steel strip to be printed.

2. The method of claim 1, **characterized in that**, after the sub-step S4 of step B, the printed patterns are collected by a code recognition module, and a pattern misplacement distance is determined by computer recognition, and then the process speed of the corresponding roller coating unit is revised.

3. The method of any of claims 1or 2, **characterized in that**, in the step A, using an decoiler to decoil and trim the steel strip and using a seamer to seam the decoiled steel strip.

4. The method of any of claims 1-3, further comprising a step of pre-processing the steel strip to be printed before transferring between the step A and the step B.

5. The method of any of claims 1-4, **characterized in that**, a recoiler is used to coil the steel strip after completing all the roller coating transfer.

6. The method of any of claims 1-5, **characterized in that**, said roller coating unit used in the step B and the step C comprises a feeding equipment (1) used for providing paints; a suction roller (2), whose circumferential surface is in connection with the feeding equipment (1) and has a plurality of recesses adapted for being filled with paints for forming an image area; a rubber-coating roller (3), with its circumferential surface in connection with the suction roller (2), used for receiving and transferring the image area formed by the paints on the coating roller (3) onto a steel plate; a first scraper (4), arranged on a first scraper support and contacting with the suction roller (2) at a specific angle, used for scraping off paints outside the image area on the suction roller (2); and a second scraper (5), arranged on the second scraper support and contacting with the coating roller (3) at a specific angle, used for scraping off paints outside the image area on the rubber coating roller (3).

## Patentansprüche

1. Verfahren zur Herstellung einer bunten Stahlplatte mit mehrfarbigen Mustern, aufweisend die folgenden Prozessschritte der Reihe nach:
A. Vorbereiten eines zu bedruckenden Stahlbandes;
B. Verwenden einer ersten Walzenbeschichtungseinheit zum Ausführen eines ersten Walzenbeschichtungstransfers auf das zu bedruckende Stahlband;
C. Verwenden einer zweiten Walzenbeschichtungseinheit zum Ausführen eines zweiten Walzenbeschichtungstransfers auf das zu bedruckende Stahlband nach einer bestimmten Zeit;
in Schritt B wird ein Servosteuersystem verwendet, um die erste Walzenbeschichtungseinheit zu steuern, und das Servosteuersystem weist den folgenden Steuerungsprozess auf:
S1. Durchmesserdaten jeder Walze und eine Prozessgeschwindigkeit der ersten Walzenbeschichtungseinheit werden in ein SPS-Steuermodul eingegeben, dann berechnet das SPS-Steuermodul die theoretische Walzenflächenlineargeschwindigkeit jeder Walze entsprechend der Prozessgeschwindigkeit und dem Durchmesser jeder Walze, berücksichtigt, dass die theoretische Walzenflächenlineargeschwindigkeit jeder Walze mit der Prozessgeschwindigkeit übereinstimmt, und gibt das berechnete theoretische Walzenflächenlineargeschwindigkeitssignal jeder Walze in ein Servosteuermodul ein, das einen Encoder aufweist;
S2. das Servosteuermodul empfängt das theoretische Walzenflächenlineargeschwindigkeitssignal jeder Walze vom SPS-Steuermodul und treibt jede Walze gemäß dem Signal an;
S3. der Encoder sammelt die tatsächliche Walzenflächenlineargeschwindigkeit jeder Walze und gibt das tatsächliche Walzenflächenlineargeschwindigkeitssignal jeder Walze an das SPS-Steuermodul aus;
S4. gemäß dem empfangenen tatsächlichen Walzenflächenlineargeschwindigkeitssignal und dem theoretischen Walzenflächenlineargeschwindigkeitssignal jeder Walze passt das SPS-Steuermodul die Stromfrequenz der elektrischen Maschine, die jede Walze antreibt, an und passt die tatsächliche Walzenflächenlineargeschwindigkeit jeder Walze so an, dass sie mit der theoretischen Walzenflächenlineargeschwindigkeit jeder Walze übereinstimmt, und dann ist der Walzenbeschichtungstransfer der ersten Walzenbeschichtungseinheit abgeschlossen;
**dadurch gekennzeichnet, dass** im Teilschritt S1 von Schritt B die Entfernungsdaten zwischen der ersten Walzenbeschichtungseinheit und der zweiten Walzenbeschichtungseinheit in das SPS-Steuermodul eingegeben werden, und das SPS-Steuermodul auf der Grundlage der Prozessgeschwindigkeit und der Entfernungsdaten eine bestimmte Zeit für den Start der zweiten Walzenbeschichtungseinheit berechnet, und die zweite Walzenbeschichtungseinheit gemäß der bestimmten Zeit startet, und dann ist der zweite Walzenbeschichtungstransfer der zweiten Walzenbeschichtungseinheit abgeschlossen;
der Walzenbeschichtungstransfer der ersten Walzenbeschichtungseinheit und der zweite Walzenbeschichtungstransfer der zweiten Walzenbeschichtungseinheit dazu verwendet werden, mehrfarbige Muster auf das zu bedruckende Stahlband zu drucken.

2. Verfahren nach Anspruch 1, **dadurch gekennzeichnet, dass** nach dem Teilschritt S4 von Schritt B die gedruckten Muster von einem Code-Erkennungsmodul gesammelt werden, und durch Computererkennung ein Musterverschiebungsabstand ermittelt wird, und dann die Prozessgeschwindigkeit der entsprechenden Walzenbeschichtungseinheit korrigiert wird.

3. Verfahren nach einem der Ansprüche 1 oder 2, **dadurch gekennzeichnet, dass** in Schritt A eine Abwickelhaspel zum Abwickeln und Abschneiden des Stahlbands und eine Nahtmaschine zum Bördeln des abgewickelten Stahlbands verwendet werden.

4. Verfahren nach einem der Ansprüche 1 - 3, ferner aufweisend einen Schritt des Vorverarbeitens des zu bedruckenden Stahlbands vor dem Transfer zwischen Schritt A und Schritt B.

5. Verfahren nach einem der Ansprüche 1 - 4, **dadurch gekennzeichnet, dass** eine Aufwickelhaspel verwendet wird, um das Stahlband nach Abschluss des gesamten Walzenbeschichtungstransfers aufzuwickeln.

6. Verfahren nach einem der Ansprüche 1 - 5, **dadurch gekennzeichnet, dass** die Walzenbeschichtungseinheit, die in Schritt B und Schritt C verwendet wird, aufweist: eine Zuführvorrichtung (1) zum Bereitstellen der Farben; eine Saugwalze (2), deren Umfangsfläche mit der Zuführvorrichtung (1) in Zusammenhang steht und die mehrere Aussparungen, die dafür geeignet sind, zur Bildung eines Bildbereichs mit Farben gefüllt zu werden, aufweist; eine Gummibeschichtungswalze (3), deren Umfangsfläche mit der Saugwalze (2) in Zusammenhang steht, die dafür verwendet wird, den von den Farben auf der Beschichtungswalze (3) gebildeten Bildbereich aufzunehmen und auf eine Stahlplatte zu übertragen; eine erste Rakel (4), die an einem ersten Rakelhalter angeordnet ist, mit der Saugwalze (2) in einem bestimmten Winkel in Kontakt steht und dafür verwendet wird, Farben außerhalb des Bildbereichs von der Saugwalze (2) abzuschaben; und eine zweite Rakel (5), die an dem zweiten Rakelhalter angeordnet ist, in einem bestimmten Winkel mit der Saugwalze (3) in Kontakt steht und dafür verwendet wird, Farben außerhalb des Bildbereichs von der Gummibeschichtungswalze (3) abzuschaben.

## Revendications

1. Procédé de production d'une plaque en acier marbrée comportant des motifs multicolores, comprenant les étapes de traitement suivantes, en séquence:
A. préparer une bande d'acier à imprimer;
B. utiliser une première unité de revêtement au rouleau pour effectuer un premier transfert de revêtement au rouleau sur la bande d'acier à imprimer;
C. utiliser une seconde unité de revêtement au rouleau pour effectuer un second transfert de revêtement au rouleau sur la bande d'acier à imprimer après un temps spécifique;
à l'étape B, un système de servocommande est utilisé pour commander ladite première unité de revêtement au rouleau, et le système de servocommande présente un processus de commande suivant:
S1. des données de diamètre de chaque rouleau et une vitesse de traitement de ladite première unité de revêtement au rouleau sont entrées dans un module de commande PLC, ensuite le module de commande PLC calcule la vitesse linéaire de surface de rouleau théorique de chaque rouleau selon la vitesse de traitement et le diamètre de chaque rouleau, rend la vitesse linéaire de surface de rouleau théorique de chaque rouleau cohérente avec la vitesse de traitement, et délivre le signal de vitesse linéaire de surface de rouleau théorique calculée de chaque rouleau dans un module de servocommande comprenant un codeur;
S2. le module de servocommande reçoit ledit signal de vitesse linéaire de surface de rouleau théorique de chaque rouleau en provenance du module de commande PLC et entraîne chaque rouleau selon le signal;
S3. le codeur collecte la vitesse linéaire de surface de rouleau réelle de chaque rouleau et délivre le signal de vitesse linéaire de surface de rouleau réel de chaque rouleau dans le module de commande PLC;
S4. selon le signal de vitesse linéaire de surface de rouleau réelle reçu et le signal de vitesse linéaire de surface de rouleau théorique de chaque rouleau, le module de commande PLC règle la fréquence de courant d'une machine électrique qui entraîne chaque rouleau, et règle la vitesse linéaire de surface de rouleau réelle de chaque rouleau de telle sorte qu'elle soit cohérente avec la vitesse linéaire de surface de rouleau théorique de chaque rouleau, et ensuite le transfert de revêtement au rouleau de la première unité de revêtement au rouleau est accompli;
**caractérisé en ce que**, à la sous-étape S1 de l'étape B, des données de distance entre la première unité de revêtement au rouleau et la seconde unité de revêtement au rouleau sont entrées dans le module de commande PLC, et sur la base de la vitesse de traitement et des données de distance, le module de commande PLC calcule un temps spécifique pour démarrer la seconde unité de revêtement au rouleau, et démarre la seconde unité de revêtement au rouleau selon le temps spécifique, et ensuite le second transfert de revêtement au rouleau de la seconde unité de revêtement au rouleau est accompli; et
le transfert de revêtement au rouleau de la première unité de revêtement au rouleau et le second transfert au rouleau de la seconde unité de revêtement au rouleau sont utilisés pour imprimer des motifs multicolores sur la bande d'acier à imprimer.

2. Procédé selon la revendication 1, **caractérisé en ce que**, après la sous-étape S4 de étape B, les motifs d'impression sont collectés par un module de reconnaissance de code, et une distance de mauvais positionnement de motif est déterminée par une reconnaissance informatique, et ensuite la vitesse de traitement de l'unité de revêtement au rouleau correspondante est révisée.

3. Procédé selon l'une quelconque des revendications 1 ou 2, **caractérisé en ce que**, à l'étape A, on utilise une dérouleuse pour dérouler et rogner la bande d'acier et on utilise une soudeuse pour souder la bande d'acier déroulée.

4. Procédé selon l'une quelconque des revendications 1 à 3, comprenant en outre une étape de prétraitement de la bande d'acier à imprimer avant le transfert entre l'étape A et l'étape B.

5. Procédé selon l'une quelconque des revendications 1 à 4, **caractérisé en ce qu'**une enrouleuse est utilisée pour bobiner la bande d'acier après l'accomplissement de la totalité du transfert de revêtement au rouleau.

6. Procédé selon l'une quelconque des revendications 1 à 5, **caractérisé en ce que** ladite unité de revêtement au rouleau utilisée dans l'étape B et l'étape C comprend un équipement d'alimentation (1) utilisé pour fournir des peintures; un rouleau d'aspiration (2) dont la surface circonférentielle est en connexion avec l'équipement d'alimentation (1) et présente une pluralité d'évidements adaptés pour être remplis avec des peintures pour former une région d'image; un rouleau de dépôt en caoutchouc (3), dont la surface circonférentielle est en connexion avec le rouleau d'aspiration (2), utilisé pour recevoir et transférer la région d'image formée par les peintures sur le rouleau de revêtement (3) sur une plaque d'acier; un premier racloir (4), agencé sur un premier support de racloir et en contact avec le rouleau d'aspiration (2) sous un angle spécifique, utilisé pour racler les peintures à l'extérieur de la région d'image sur le rouleau d'aspiration (2); et un second racloir (5), agencé sur le second support de racloir et en contact avec le rouleau de revêtement (3) sous un angle spécifique, utilisé pour racler les peintures à l'extérieur de la région d'image sur le rouleau de dépôt en caoutchouc (3).
